

J. O. HEINZE, JR.

METHOD OF TREATING METAL STRUCTURES TO PREVENT SUBSEQUENT CHANGE IN FORM.  
APPLICATION FILED APR. 9, 1912.

1,132,262.

Patented Mar. 16, 1915.



Witnesses  
W. K. Ford  
James A. Barry

Inventor  
John O. Heinze, Jr.  
By Whittmore, Hubbard & Whittmore  
Atty's.

# UNITED STATES PATENT OFFICE.

JOHN O. HEINZE, JR., OF DETROIT, MICHIGAN, ASSIGNOR TO GENERAL MOTORS COMPANY, OF DETROIT, MICHIGAN, A CORPORATION OF MICHIGAN.

## METHOD OF TREATING METAL STRUCTURES TO PREVENT SUBSEQUENT CHANGE IN FORM.

1,132,262.

Specification of Letters Patent. Patented Mar. 16, 1915.

Application filed April 9, 1912. Serial No. 689,603.

*To all whom it may concern:*

Be it known that I, JOHN O. HEINZE, Jr., a citizen of the United States of America, residing at Detroit, in the county of Wayne and State of Michigan, have invented certain new and useful Improvements in Methods of Treating Metal Structures to Prevent Subsequent Change in Form, of which the following is a specification, reference being had therein to the accompanying drawings.

The invention relates to the manufacture of machined parts where it is necessary to the proper operation to maintain an exact form, such for instance as the pistons and cylinders of engines. Such structures are usually formed of cast metal, and as an incident to the cooling molten metal during the casting process, unequal stresses are set up in the metal. These stresses may be partially relieved by the removal of the scale in roughing out the structure, but experience has demonstrated that until the metal is subjected to work analogous to that which it performs in the complete structure, these stresses are not entirely equalized. As a consequence the pistons may be ground or otherwise fashioned to exactly fit the cylinder, but after the machine has been in operation for a short time the form will change.

My invention is designed to overcome this difficulty by magnetically agitating the molecules of the metal before the casting is fashioned, thereby equalizing the stresses and preventing subsequent change in form.

My method of treatment may be carried out in various ways, but as shown,

In the drawings,—Figure 1 is a sectional elevation of one form of apparatus; Fig. 2 is a horizontal section therethrough; and Fig. 3 is a diagrammatic view showing the magnetic connections.

A is a core of laminated magnetic metal which is preferably in the form of a continuous ring.

B is a helix or solenoid which is insertible within the ring A and which is adapted to receive the metal to be treated.

As shown, the structure which is treated is a piston C the length of which corresponds to the distance between the opposite poles D and E of the ring A, whereby a complete magnetic circuit will be formed when the helix or solenoid B is energized.

The process of treatment is to first insert 55 the casting C into the helix B, then to place said helix and core within the ring A, after which an alternating electric current is passed through the helix or solenoid. This will produce magnetic vibrations within the 60 metal C which will relieve the condition of unequal stress and permit the metal to assume a form which will be permanently retained.

After the treatment the casting is removed 65 and is machined and ground or otherwise fashioned to the desired form.

To guard against any stress or tension in the metal that may be set up through the operation of machining I preferably subject 70 the casting to a treatment after the roughing out cut has been taken, but before the grinding or other finishing operation, and in some instances it may be desirable to subject the metal to a plurality of treatments, 75 first in the rough and then after each machine cut.

For convenience in manipulation the helix B is provided with a handle F by which it may be inserted or withdrawn and the electric connections to the circuit G including the alternating current generator H, may be completed through this handle.

What I claim as my invention is:

1. The process of treating metal to equalize molecular stresses therein which consists in subjecting the same at normal temperature to magnetic fluctuations.

2. The process of treating metal at normal temperature to equalize molecular stresses therein which consists in including the metal to be treated within a magnetic circuit and producing magnetic fluctuations in said circuit.

3. The process of treating metal at normal temperature to equalize molecular stresses therein which consists in placing the metal to be treated in a magnetic circuit and in producing magnetic fluctuations in said circuit by an alternating electric current.

4. The process of treating metal at normal temperature to equalize molecular stresses therein which consists in surrounding the metal to be treated by a helix or solenoid, in completing the magnetic circuit 105 between the opposite ends of the metal within said helix, and in passing a fluctuating electric current through the helix to produce

corresponding magnetic fluctuations in the metal treated.

5. The method of treating solid metal to alter its molecular structure, consisting in temporarily subjecting it to the action of the magnetic field of an alternating current.

6. The method of treating solid metal to alter its molecular structure, consisting in placing said metal adjacent to a conductor carrying an alternating current, subjecting it to the action of the magnetic field of said current until the desired result is obtained, and then removing it therefrom.

10 7. The method of treating solid metal to

alter its molecular structure, consisting in 15 placing it within a coil, passing an alternating current through said coil, and subjecting the metal to the action of the magnetic field of said alternating current until the desired effect is obtained, and then removing 20 it therefrom.

In testimony whereof I affix my signature in presence of two witnesses.

JOHN O. HEINZE, JR.

Witnesses:

JAMES P. BARRY,  
DELBERT COLLINS.